

Sept. 30, 1958

R. S. ROSE

2,854,331

ALLOYS AND ALLOY ARTICLES

Filed Oct. 26, 1956

$$P_{25} \times 10^3 = T (25 + \log t)$$



INVENTOR

Robert S. Rose

*For  
Robert S. Rose  
Attorney*

# United States Patent Office

2,854,331

Patented Sept. 30, 1958

1

2,854,331

## ALLOYS AND ALLOY ARTICLES

Robert S. Rose, Waban, Mass., assignor to Latrobe Steel Company, Latrobe, Pa., a corporation of Pennsylvania

Application October 26, 1956, Serial No. 618,424

4 Claims. (Cl. 75—128)

This invention relates to alloys and alloy articles and particularly to an alloy and alloy article having substantially improved hardness and stress-rupture properties at elevated temperature without any impairment of ductility.

There has long been a need for a steel alloy having a high degree of hardness and high stress-rupture properties at elevated temperatures while at the same time retaining a high degree of ductility. This need has been accentuated by the demands of the jet engine and high temperature turbine fields. There are presently available no alloys having all of these properties.

I provide an alloy whose composition is broadly as follows:

W about 1%—5%

Ni about .75%—2.75%

Cr about 10%—17%

Cb about .3%—1%

C about .10%—.25% plus an amount equal to 10% of the amount of columbium present

Mn less than about 1.5%

Si less than about 1.5%

Fe balance with usual impurities in ordinary amounts.

Preferably, I limit the alloy to a somewhat narrower range as follows:

W about 2.75%—3.25%

Ni about 1.75%—2.25%

Cr about 12.5%—13.5%

Cb about .30%—.40%

C about .12%—.20% plus an amount equal to 10% of the amount of columbium present

Mn less than about 1.5%

Si less than about 1.5%

Fe balance with usual impurities in ordinary amounts.

The beneficial effect of this new discovery on elevated temperature hardness when compared to an alloy now generally used but without the presence of columbium and added carbon as taught herein is shown in Table I.

TABLE I

Heat treating modified and regular tungsten stainless iron material:  $\frac{1}{2}$ " thick discs. Prior condition: annealed

[All samples were austenitized by holding at the indicated temperature 30 minutes, then oil quenching—all tempers were of 2 hours duration.]

## MODIFIED TUNGSTEN STAINLESS IRON

| Austenitizing Temperature, °F. | As Quenched | Hardness—Rockwell C |           |           |           |
|--------------------------------|-------------|---------------------|-----------|-----------|-----------|
|                                |             | 1,000° F.           | 1,100° F. | 1,200° F. | 1,300° F. |
| 1,800                          | 49.6        | 39.1                | 34.0      | 31.5      | 30.3      |
| 1,850                          | 50.5        | 39.9                | 34.5      | 32.2      | 30.8      |
| 1,900                          | 51.0        | 40.5                | 35.0      | 33.1      | 32.2      |
| 1,950                          | 50.9        | 41.4                | 35.1      | 33.0      | 32.0      |
| 2,000                          | 51.3        | 42.1                | 36.2      | 34.5      | 32.9      |
| 2,050                          | 51.4        | 42.7                | 37.2      | 35.0      | 33.9      |
| 2,100                          | 51.1        | 42.9                | 37.4      | 35.5      | 34.5      |

## REGULAR TUNGSTEN STAINLESS IRON

|       |      |      |      |      |      |
|-------|------|------|------|------|------|
| 1,800 | 49.3 | 39.1 | 33.2 | 29.2 | 28.0 |
| 1,850 | 51.3 | 40.9 | 33.8 | 29.9 | 28.9 |
| 1,900 | 50.9 | 40.7 | 32.3 | 29.4 | 28.8 |
| 1,950 | 50.8 | 40.6 | 33.6 | 29.5 | 28.3 |
| 2,000 | 50.7 | 40.9 | 33.4 | 30.3 | 28.7 |
| 2,050 | 50.5 | 40.2 | 33.5 | 29.5 | 28.2 |
| 2,100 |      |      |      |      |      |

2

Stress rupture properties are among the most important for aircraft gas turbine and compressor application. Table II sets forth the rupture strength, elongation and reduction of area of this new composition. For comparison Table III gives values for the base alloy. The substantial improvement is evident upon study of the data.

TABLE II

## Rupture strength of modified tungsten stainless iron

| S. R. | Stress (p. s. i. $\times 10^3$ ) | Temperature, °F. | R. L. (hrs.) | Percent Elongation | Percent Reduction of Area | P25   |
|-------|----------------------------------|------------------|--------------|--------------------|---------------------------|-------|
| 934   | 95                               | 1,000            | 0.05         | 12.8               | 51.5                      | 34.47 |
| 929   | 75                               | 1,000            | 66.6         | 15.4               | 54.0                      | 39.02 |
| 939   | 75                               | 1,000            | 48.5         | 24.2               | 60.0                      | 38.82 |
| 833   | 70                               | 1,000            | 276.9        | 16.2               | 53.5                      | 39.92 |
| 940   | 65                               | 1,050            | 79.1         | 19.2               | 67.0                      | 40.47 |
| 834   | 60                               | 1,050            | 117.2        | 28.3               | 65.4                      | 40.73 |
| 941   | 55                               | 1,100            | 181.2        | 16.0               | 68.7                      | 42.38 |
| 835   | 50                               | 1,100            | 114.2        | 14.8               | 57.3                      | 42.06 |
| 932   | 40                               | 1,150            | 121.4        | 16.1               | 65.0                      | 43.46 |
| 937   | 40                               | 1,150            | 78.8         | 14.5               | 57.7                      | 43.16 |
| 942   | 40                               | 1,150            | 161.3        | 24.5               | 65.5                      | 43.66 |
| 837   | 30                               | 1,200            | 116.3        | 21.4               | 72.6                      | 44.78 |
| 933   | 30                               | 1,200            | 54.1         | 24.8               | 71.2                      | 44.23 |
| 938   | 30                               | 1,200            | 56.8         | 23.4               | 66.0                      | 44.27 |
| 943   | 30                               | 1,200            | 88.2         | 19.1               | 71.5                      | 44.58 |

Samples treated 2000° F., oil quenched

Temper 1200° F.

Hardness—Rockwell C 34

TABLE III

## Rupture strength of regular tungsten stainless iron

| S. R. | Stress (p. s. i. $\times 10^3$ ) | Temp., °F. | R. L. (hrs.) | Percent Elongation | Percent Reduction of Area | P25   | Heat  |
|-------|----------------------------------|------------|--------------|--------------------|---------------------------|-------|-------|
| 987   | 75                               | 1,000      | 0.62         | 18.9               | 67.5                      | 36.06 | 47943 |
| 991   | 75                               | 1,000      | 0.47         | 17.1               | 70.9                      | 35.89 | 47943 |
| 993   | 70                               | 1,000      | 13.00        | 18.5               | 71.4                      | 37.99 | 52007 |
| 992   | 65                               | 1,050      | 4.5          | 21.6               | 68.3                      | 38.60 | 52007 |
| 988   | 65                               | 1,050      | .30          | 16.5               | 65.6                      | 36.83 | 47943 |
| 994   | 65                               | 1,000      | 265.2        | 20.5               | 67.3                      | 39.89 | 52007 |
| 939   | 55                               | 1,100      | 0.67         | 22.9               | 75.7                      | 38.60 | 47943 |
| 995   | 55                               | 1,050      | 162.4        | 13.5               | 61.6                      | 40.94 | 52007 |
| 990   | 40                               | 1,150      | 5.2          | 20.3               | 77.8                      | 41.26 | 47943 |
| 840   | 40                               | 1,100      | 134.0        | 18.1               | 64.7                      | 42.17 | 36789 |
| 844   | 40                               | 1,100      | 130.6        | 13.3               | 58.9                      | 42.15 | 36789 |
| 847   | 40                               | 1,100      | 161.7        | 20.6               | 59.8                      | 42.30 | 36789 |
| 996   | 40                               | 1,100      | 315.8        | 11.7               | 57.0                      | 42.75 | 52007 |
| 841   | 30                               | 1,160      | 101.5        | 18.2               | 59.0                      | 43.61 | 36789 |
| 845   | 30                               | 1,160      | 43.4         | 27.6               | 75.5                      | 43.01 | 36789 |

Samples treated 1850° F., oil quenched

Temper 1100° F.

Hardness—Rockwell C 34

To enable a direct comparison of three variables: rupture strength, time, and temperature, on a two dimensional chart, a stress parameter formula has been used.

$$P_{25} \times 10^3 = T(25 + \log t)$$

Where:

60 25 is a constant for 12% chrome alloys

T is absolute temperature ° F.

t is time

The significant increase in elevated temperature properties is clearly obvious in the figure. This figure is a comparison of the stress-parameter of a regular tungsten stainless and an alloy according to the present invention. Comparisons along verticals 39 and 40 show a 20% improvement in stress-parameter for the new discovery.

70 While I have set forth certain preferred compositions and alloy articles of this invention in the foregoing specification, it will be understood that this invention

may be otherwise embodied within the scope of the following claims:

I claim:

1. A ferrous alloy of high hardness and stress-rupture properties at elevated temperatures comprising about .10% to .25% carbon plus an amount of carbon equal to 10% of the columbium present, about 10% to 17% chromium, from 1% to 5% tungsten, about .75% to 2.75% nickel, about .3% to 1% columbium, less than about 1.5% manganese, less than about 1.5% silicon and the balance substantially iron with residual impurities in ordinary amounts.

2. A ferrous article formed from a ductile heat and corrosion resistant ferrous alloy comprising about .10% to .25% carbon plus an amount of carbon equal to 10% of the columbium present, about 10% to 17% chromium, about 1% to 5% tungsten, about .75% to 2.75% nickel, about .3% to .1% columbium, less than about 1.5% manganese, less than about 1.5% silicon and the balance substantially iron with residual impurities in ordinary amounts, said article being characterized by a high degree of hardness and high stress-rupture properties at elevated temperatures along with a high degree of ductility.

3. A ferrous alloy of high hardness and stress-rupture properties at elevated temperatures comprising about .12% 25

to .20% carbon plus an amount of carbon equal to 10% of the columbium present, about 12.5% to 13.5% chromium, from 2.75% to 3.25% tungsten, about 1.75% to 2.25% nickel, about .3% to .4% columbium, less than about 1.5 manganese, less than about 1.5% silicon and the balance substantially iron with residual impurities in ordinary amounts.

4. A ferrous article formed from a ductile heat and corrosion resistant ferrous alloy comprising about .12% to .20% carbon plus an amount of carbon equal to 10% of the columbium present, about 12.5% to 13.5% chromium, about 2.75% to 3.25% tungsten, about 1.75% to 2.25% nickel, about .3% to .4% columbium, less than about 1.5% manganese, less than about 1.5% silicon and the balance substantially iron with residual impurities in ordinary amounts, said article being characterized by a high degree of hardness and high stress-rupture properties at elevated temperatures along with a high degree of ductility.

References Cited in the file of this patent

UNITED STATES PATENTS

|           |                   |              |
|-----------|-------------------|--------------|
| 2,227,891 | Rose -----        | Jan. 7, 1941 |
| 2,793,113 | Rait et al. ----- | May 21, 1957 |